# EUROPEAN PATENT SPECIFICATION

(11) **EP 1 834 009 B1**
(45) Date of publication and mention of the grant of the patent: **20.07.2016**
(21) Application number: 05853894.3
(22) Date of filing: 12.12.2005
(51) Int. Cl.: C23C 18/06, C23C 18/12, C23C 22/48, C23C 22/74

(54) **METAL COMPONENTS WITH SILICON-CONTAINING PROTECTIVE COATINGS AND METHODS OF FORMING SUCH PROTECTIVE COATINGS**
METALLTEILE MIT SILIZIUMHALTIGEN SCHUTZSCHICHTEN UND VERFAHREN ZUR BILDUNG SOLCHER SCHUTZSCHICHTEN
COMPOSANTS METALLIQUES AVEC REVETEMENTS PROTECTEURS AU SILICIUM ET PROCEDES DE FORMATION DE CES REVETEMENTS PROTECTEURS

(30) Priority: 13.12.2004 WO PCT/US2004/041896
(43) Date of publication of application: 19.09.2007
(62) Divisional of application: 16171410.0
(73) Proprietor: MT Coatings, LLC, Cincinnati, OH 45225 (US)
(72) Inventor: FAIRBOURN, David, C., Sandy, Utah 84093 (US)
(74) Representative: Eisenführ Speiser
(86) International application number: PCT/US2005/045078
(87) International publication number: WO 2006/065819

(56) References cited:
- EP-A- 0 327 311
- WO-A-98/30735
- WO-A-02/099153
- WO-A-03/035942
- WO-A-2006/036171
- GB-A- 893 397
- US-A- 4 500 364
- US-A1- 2003 185 990

## Description

### Field of the Invention

The present invention relates to coated metal components and, more particularly, substantially chromium-free metal components with a substantially chromium-free protective coating containing silicon, and methods of forming such substantially chromium-free protective coatings on substantially chromium-free metal components.

### Background of the Invention

Inorganic layers and coatings are often formed on a surface of a substantially chromium-free metal component to protect and mask the underlying metal substrate and to extend its useful life, such as by providing corrosion resistance and chemical resistance. Although zinc may be applied as an inorganic protective coating on iron or steel substrates either electrochemically by plating or by hot dip methods, such zinc protective coatings may be subject to corrosion in the form of a white rust defect. To prevent the occurrence of white rust defects, a conversion coating such as a chromate may be applied as a pretreatment on the iron or steel substrate before the zinc is applied. However, the process forming chromate coatings presents environmental and health risks that reduce their prevalence of use and that have instigated research to identify suitable substitute environmentally friendly coatings to replace chromate coatings.

Hard chrome plating is another common inorganic protective coating used in industrial equipment to reduce friction and wear. Hard chrome coatings are applied by electrolytic deposition processes. However, electrolytic deposition processes involve chemicals that are extremely hazardous, toxic, corrosive, and damaging to the environment. The use, storage, and disposal of the chemicals involved in electrolytic deposition processes are governed by law in most jurisdictions. Personal safety equipment and proper containment facilities are considered mandatory.

Copper is most frequently used as a pure, unalloyed metal. For example, copper tubing and pipes are used to transport potable water in a residence. However, copper corrodes over time and, if sulfur has been present, turns blue due to the formation of copper sulfate from sulfur exposure.

Organic (i.e., carbon-based) coatings, such as conventional paints, may also be used to protect substantially chromium-free metal substrates. However, organic coatings may deteriorate at high temperatures because of the presence of a polymer operating as a binder to confer film-forming properties. Consequently, organic coatings may lose their protective ability such that the formerly protected metal substrate is vulnerable to corrosion or chemical attack.

### Summary of the Invention

The present invention provides a coating process for protecting a surface of a substantially chromium-free metal component, comprising applying a layer of a substantially chromium-free, silicon-containing fluid composition comprising a silane liquid to at least a portion of the surface, curing the substantially chromium-free, silicon-containing fluid composition after the layer is applied to the surface, placing the silicon-containing fluid composition in a non-oxidizing atmosphere and then heating the cured substantially chromium-free, silicon-containing fluid composition in layer in the non-oxidising atmosphere to a temperature greater than 400°F (204.44°C) to form a substantially chromium-free, silicon-containing protective coating on the surface that includes silicon from the cured silicon-containing fluid composition and metal from the metal component. The protective coating may be, for example, effective for reducing corrosion and sulfidation of the underlying metal of the metal comopnent. The metal component may be formed from any metal including, but not limited to, iron, aluminum, titanium, copper, nickel, and alloys of each of these metals such as mild steel and stainless steels.

The properties of the protective coating may be tailored according to the type of atmosphere in which the substantially chromium-free, silicon-containing fluid composition layer is heated. The fluid composition layer may be heated in argon to form, for example, a metal silicide protective coating.

The substantially chromium-free, silicon-containing protective coating of the present invention would operate to mask and protect the underlying base metal of the metal component at room temperature and may retain the protective properties at elevated temperatures that area significantly above room temperature. The heat resistance would be advantageous in comparison to, for example, conventional organic or carbon-based paints that deteriorate at high temperatures and, therefore, lose their protective ability.

The protective coating of the present invention would also eliminate the risks and concerns associated with producing conventional chromate coatings and hard chromium plating, among other types of conventional coatings. The protective coating of the present invention may also be applied to metal components that otherwise would not receive such coatings, such as copper tubing. The protective coating of the present invention may also reduce the need to alloy the metal of a component with another metal to impart corrosion resistance.

These and other benefits and advantages of the present invention shall be made apparent from the accompanying drawings and description thereof.

### Brief Description of the Drawings

The accompanying drawings, which are incorporated in and constitute a part of this specification, illustrate an embodiment of the invention and, together with a general description of the invention given above, and the detailed description of the embodiment given below, serve to explain the principles of the invention.
**Fig. 1** is a perspective view of a metal component with a fluid composition being applied to at least a portion of the metal component in accordance with the principles of the present invention;
**Fig. 2** is a diagrammatic cross-sectional view of a portion of the metal component of **Fig. 1** that includes a silicon-containing layer formed by the application of the fluid composition;
**Fig. 2A** is a diagrammatic cross-sectional view similar to **Fig. 2** in which the silicon-containing layer is applied on an existing layer on the metal component; and
**Fig. 3** is a diagrammatic cross-sectional view similar to **Fig. 2** after the silicon-containing layer is converted to a protective coating.

### Detailed Description of Preferred Embodiments

With reference to **Figs. 1** and **2** and in accordance with an embodiment of the present invention, a substantially chromium-free, silicon-containing layer 12 is applied to at least a portion of an original surface 14 of a substantially chromium-free metal component 10. The metal component 10 may be formed from a substantially chromium-free substrate 15 that includes any metal including, but not limited to, iron, aluminum, titanium, copper, nickel, and alloys of each of these materials, including mild steel and stainless steels. The metal may also include some non-metallic components. However, layer 12 and substrate 15 are substantially free of chromium content, other than a trace amount of chromium present as an impurity.

The substantially chromium-free, silicon-containing layer 12 is formed from a substantially chromium-free, silicon-containing fluid composition (e.g., liquid composition, solution, or slurry) that is applied to surface 14, such as by hand application with a paint brush B **(****Fig. 1****)** as if being painted, by spraying in a controlled manner, or by dipping into a bath (not shown). The uncured fluid composition is then cured at a low temperature to form a solid or semi-solid that is bonded to the surface 14. In one embodiment of the present invention, the silicon-containing layer 12 may be cured by air-drying with optional heating. The curing temperature of the silicon-containing layer 12 is significantly less than 400°F (204.44 °C). For example, the fluid composition may be cured at about 250°F (121°C) for about 15 to 25 minutes to form the silicon-containing layer 12. The fluid composition forming layer 12 is substantially free of chromium content, other than a trace amount of chromium present as an impurity.

Before the substantially chromium-free, silicon-containing layer 12 is applied, the surface 14 may be substantially cleaned of any contaminants. For example, a degreaser, such as acetone, sodium hydroxide (NaOH) or potassium hydroxide (KOH) may be used to clean the surface 14 and potentially improve the bonding of the cured layer 12 to the surface. A biocide, such as silver chloride (AgCl) may also be added to the fluid composition before layer 12 is applied to surface 14.

A particular fluid or liquid composition that may be selected for use in forming layer 12 comprises a silane liquid. Silanes suitable for use in the present invention may have mono-, bis-, or tri-functional trialkoxy silane. The silane may be a bifunctional trialkoxy silyl, preferably trimethoxy, or triethoxy silyl groups. Amino silanes may also be used, although thio silanes may not be desired due to their sulfur content. Bisfunctional silane compounds are well known to persons having ordinary skill in the art, and two preferred for use in the present invention are bis(triethoxysilyl) ethane and bis(trimethoxysilyl) methane. In both of these compounds, the bridging group between the two silane moieties is an alkyl group. Additional commercially available silanes include, but are not limited to,
1, 2- Bis(tetramethyldisoloxanyl) Ethane
1, 9- Bis(triethoxysilyl) Nonane
Bis(triethoxysilyl) Octane
Bis(trimethoxysilyl Ethane
1, 3- Bis(trimethylsiloxy)-1,3-Dimethyl Disiloxane
Bis(trimethylsiloxy) Ethylsilane
Bis(trimethylsiloxy) Methylsilane
Al-501 available from AG Chemetall (Frankfurt Germany)

The silane may be neat, in an aqueous solution, or diluted in an aqueous/alcohol solvent solution. A solvent for the latter type of diluted solution may contain from about 1% to 2% by volume to about 30% by volume deionized water with the remainder being a monohydric alcohol such as methanol, ethanol, n- or iso-propanol, or the like. Ethanol and methanol are preferred monohydric alcohols. The solvent is combined with the silane and glacial acetic acid to preferably establish a pH of about 4-6. The silane concentration in the solution may be limited to a maximum concentration for which the silane remains in solution during application. Generally, the solution will consist of about 1% to about 20% silane, wherein the percentage may be measured either by volume or by weight.

A particularly useful silane for use in providing silicon-containing layer 12 may be an organofunctional silane such as BTSE 1,2 bis(triethoxysilyl) ethane or BTSM 1,2 bis(trimethoxysilyl) methane. The silane may be dissolved in a mixture of water and acetic acid at a pH of 5, then in denatured alcohol and glacial acetic acid to establish a silane solution. The silane concentration in the solution is between about 1% and 10% by volume and, advantageously, about 5% by volume. This silane solution readily forms the silicon-containing layer 12, which may have a more or less hard consistency, at a temperature readily achieved and insufficient to form the protective coating 16.

Generally, the liquid composition that is applied to, after curing, form the silicon-containing layer 12 is applied in an amount of about 0.01 g/cm² to about 2.0 g/cm². Multiple layers of the liquid composition may be applied; each individual layer being dried and heated to remove the solvent before applying the next successive layer. As used herein, the silicon-containing layer 12 may refer to either the initially applied layer of liquid composition, or without limitation to the dried layer. The silicon-containing layer 12 may have a thickness in the range of about 40 nm to about 200 nm in the cured state and may form a continuous layer on surface 14, although the invention is not so limited.

Silicon-containing layer 12 is heated to a temperature and for a duration effective to convert layer 12 into a substantially chromium-free, silicon-containing protective coating 16 across the portion of the original surface 14 of the metal component 10 to which layer 12 is applied. Generally, the conversion temperature is a temperature between 400°F (204.44°C) and about 70 percent of the melting temperature of the substantially chromium-free metal constituting component 10. The specific temperature to which silicon-containing layer 12 is heated to cause the conversion to protective coating 16 will depend, among other things, upon the composition and characteristics of the liquid composition used to form layer 12 and the specific metal constituting the metal component 10. The protective coating 16 may be continuous with a thickness measured relative to an exposed surface 24 that, after the coating 16 is applied, is exposed to the operating environment of the metal component 10. The protective coating 16 substantially free of chromium content, other than a trace amount of chromium present as an impurity.

A particularly advantageous conversion temperature may be the eutectic temperature for silicon and the particular metal constituting the metal component 10. A eutectic or eutectic mixture is a mixture of two or more elements that has a lower melting point than any of its constituents. The proper ratio of silicon and metal to obtain a eutectic alloy is identified by the eutectic point on a phase diagram. The eutectic point is the point at which the liquid phase borders directly on the solid forms of pure silicon and the pure metal, which represents the minimum melting temperature or eutectic temperature of any possible alloy of silicon and the metal(s) constituting the metal component 10.

The substantially chromium-free silicon-containing layer 12 is heated in a non-oxidizing atmosphere and under various different conditions to form the substantially chromium-free protective coating 16. The conversion from substantially chromium-free, silicon-containing layer 12 to substantially chromium-free, silicon-containing protective coating 16 may be accomplished by placing the metal component 10 into a heated enclosure, like an oven or furnace. However, the specific heating method may be selected based upon the size of the component 10 and the availability of heating options. The heated enclosure is heated to a temperature sufficient to elevate layer 12 to a temperature sufficient to cause the conversion. The curing step to form silicon-containing layer 12 and the subsequent step converting the cured layer 12 into protective coating 16 may be conducted in the same heated enclosure or before placing the metal component 10 into the heated enclosure. The silicon-containing layer 12 cures at a lower temperature than the temperature required to convert layer 12 into protective coating 16.

For example, the heat tunnels used in powder coaters (not shown) may provide a suitable heated environment or enclosure. In particular, this approach may be particularly advantageous for forming the protective coating 16 on metal components composed of aluminum.

The substantially chromium-free silicon-containing layer 12 is heated in a non-oxidizing ambient atmosphere, such as argon, to form a substantially chromium-free protective coating 16, such as a metal silicide, that contains silicon from layer 12 and a concentration of one or more elements from the constituent material of the metal component 10. The non-oxidizing ambient environment may be an oxygen-depleted environment created by evacuating atmospheric gases (air) from a heating chamber and filling the evacuated chamber with an inert gas.

In an alternative embodiment of the present invention, the substantially chromium-free silicon-containing layer 12 may further include an additive that is subsequently incorporated as an optional dopant into the substantially chromium-free protective coating 16. Suitable additives generally include any compound of the dopant that is dissolvable in the particular silane solution, although additives containing sulfur ligands and/or oxygen ligands may be disfavored. If the dopant is yttrium, for example, suitable yttrium compounds include, but are not limited to, yttrium halides, such as yttrium chloride, yttrium bromide, yttrium iodide, and yttrium fluoride. Other suitable yttrium compounds include, but are not limited to, yttrium acetate, yttrium acetate hydrate, yttrium 2-ethylhexanoate, yttrium perchlorate solution (e.g., 40 wt. % in water), yttrium nitrate hexahydrate, yttrium nitrate tetrahydrate, yttrium isopropoxide oxide, yttrium isopropoxide solution (e.g., 25 wt. % in toluene), yttrium butoxide solution (e.g., 0.5 M in toluene), yttrium trifluoroacetate hydrate, yttrium oxalate hydrate, and yttrium(III) tris(2,2,6,6-tetramethyl-3,5-heptanedionate). If the dopant is hafnium, for example, suitable hafnium compounds include, but are not limited to, hafnium halides, such as hafnium chloride, hafnium bromide, hafnium iodide, and hafnium fluoride. Other suitable hafnium compounds include, but are not limited to, any hafnium compound with an organic ligand, such as hafnium tert-butoxide, and hafnium nitrates. Permitted hafnium compounds generally exclude compounds with either sulfur ligands or oxide ligands. These, and other, yttrium and hafnium compounds are commercially available, for example, from Sigma-Aldrich (St. Louis, Missouri).

In this alternative embodiment of the present invention, one or more of the candidate dopant compounds is dissolved in or combined with the silane or silane solution. Before combining, the added amount of the dopant compound is measured for accurately regulating the concentration of dopant in the substantially chromium-free silicon-containing layer 12 and, subsequently, in the protective coating 16. Typically, a single additive or dopant compound will be combined with the silane to form the fluid composition that is applied as layer 12 to all or a portion of surface 14.

With reference to **Fig. 2A****,** the substantially chromium-free silicon-containing layer 12 may be applied across an existing coating 18 on substrate 15. The existing coating 18 may be, for example, an existing protective coating 16 that is in need of repair. The existing coating 18 may be stripped from surface 14 before the silicon-containing layer 12 is applied for forming the protective coating 16.

With reference to **Fig. 3****,** a detailed view of a portion of the substantially chromium-free metal component 10 and the substantially chromium-free protective coating 16 is shown. The metal component 10 includes the protective coating 16 on the surface 14 of the substrate 15. The protective coating 16 protects the underlying metal of the substrate 12 of metal component 10 against, for example, oxidation and corrosion.

The substantially chromium-free protective coating 16 is an additive layer 20 which includes a concentration of one or more elements from substrate 15 because of interdiffusion between the applied silicon-containing layer 12 and the metal of the substrate 15. In such diffusion coatings, the protective coating 16 will be generally characterized by a diffusion zone 22 in addition to the additive layer 20 that overlies the diffusion zone 22. The interdiffusion may advantageously introduce a concentration of one or more additional elements from the substrate 15 into the protective coating 16 that ultimately endow the coating 16 with beneficial protective capabilities.

The invention further contemplates that the fluid compositions described herein may be introduced into internal passages (not shown) of the substantially chromium-free metal component 10 for purposes of forming the substantially chromium-free, silicon-containing protective coating 16 on internal surfaces bordering the passages. To that end, the silicon-containing fluid composition is introduced into the passages to form substantially chromium-free, silicon-containing layer 12 and heated to form the protective coating 16 on these internal surfaces.

As an example not in accordance with the invention, the substantially chromium-free, silicon-containing layer 12 may be applied to a metal component 10 composed of zinc and heated in an oxidizing environment, like air, to a temperature greater than 400°F (204.44 °C) that is sufficient to form a protective coating 16, which may be zinc oxide, that incorporates silicon from the liquid composition constituting layer 12. Although not wishing to be limited by theory, the protective coating is believed to reduce oxidation of the underlying zinc substrate 15.

As another example, the substantially chromium-free, silicon-containing layer 12 may be applied to a metal component 10 composed of copper by immersion in the liquid composition, preferably almost immediately after the copper component 10 is drawn to a final dimension. When heated to a temperature of, for example, less than 400°C (752°F) but greater than 400°F (204.44 °C) in a non-oxidizing environment, a protective coating 16 containing silicon is formed in which silicon is incorporated into copper metal as a diffusion zone 22 with an optional additive layer 20. The protective coating 16 may be a copper silicide layer.

As yet another example, the substantially chromium-free, silicon-containing layer 12 may be applied to a metal component 10 composed of a steel. The application of a thin layer of silane followed by heating to a temperature less than 770°C (1418°F) but greater than 400°F (204.44 °C) in a non-oxidizing environment forms a protective coating 16, which may be ferric silicide, that improves corrosion resistance. The solubility of the silicon in iron is less than four (4) weight percentage. In very dilute solutions less than 0.4 weight percent silicon, silicon may replace carbon in the steel.

In another embodiment not in accordance with the invention, the existing layer 18 (Fig. 2A) may be a hard chromium coating or plating that is pre-existing on the substantially chromium-free metal component 10 before the substantially chromium-free, silicon-containing layer 12 is applied. The silicon-containing layer 12 is heated to a temperature less than 800°C (1472°F) but greater than 400°F in an inert environment to form the protective coating 16. The chromium in coating 16 does not originate from either component 10 or layer 12 but, instead, originates from layer 18.

As yet another example, the substantially chromium-free, silicon-containing layer 12 may be applied to a metal component 10 composed of aluminum, followed by heating to less than 400°C (752°F) but greater than 400°F (204.44°C) in a non-oxidizing environment, which is believed to produce a protective coating 16 of aluminum silicide. The solubility of silicon in aluminum is limited to a maximum of one (1) weight percent to 1.5 weight percent at the eutectic temperature of 577°C (1071 °F).

The protective coating 16 may also increase the resistivity of the metal of the metal component 10, which may represent an additional benefit of the present invention.

While the present invention has been illustrated by the description of an embodiment thereof and specific examples, and while the embodiment has been described in considerable detail, additional advantages and modifications will readily appear to those skilled in the art. is:

## Claims

1. A coating process for protecting a surface (14) of a substantially chromium-free metal component (10), comprising applying a layer (12) of a substantially chromium-free, silicon-containing fluid composition comprising a silane liquid to at least a portion of the surface (14), curing the substantially chromium-free, silicon-containing fluid composition after the layer (12) is applied to the surface (14), placing the silicon-containing fluid composition in a non-oxidizing atmosphere and then heating the cured substantially chromium-free, silicon-containing fluid composition in layer (12) in the non-oxidising atmosphere to a temperature greater than 400°F (204.44°C) to form a substantially chromium-free, silicon-containing protective coating (16) on the surface (14) that includes silicon from the cured silicon-containing fluid composition and metal from the metal component (10).

2. The coating process of claim 1 further comprising combining the silane liquid with a dopant selected from the group consisting of yttrium, hafnium, and combinations thereof.

3. The coating process of either claim 1 or claim 2 wherein the substantially chromium-free metal component (10) is composed of iron, aluminium, titanium, copper, nickel, or an alloy of these materials.

## Patentansprüche

1. Beschichtungsverfahren zum Schützen einer Oberfläche (14) einer im Wesentlichen chromfreien Metallkomponente (10), umfassend Auftragen einer Schicht (12) einer im Wesentlichen chromfreien, Silizium enthaltenden Fluidkomposition, die eine Siliziumwasserstoff-Flüssigkeit umfasst, auf zumindest einen Teil der Oberfläche (14), Trocknen der im Wesentlichen chromfreien, Silizium enthaltenden Fluidkomposition nachdem die Schicht (12) auf die Oberfläche (14) aufgetragen wurde, Einbringen der Silizium enthaltenden Fluidkomposition in eine nicht-oxydierende Atmosphäre und dann Erhitzen der getrockneten, im Wesentlichen chromfreien, Silizium enthaltenden Fluidkomposition in der Schicht (12) in der nicht-oxydierenden Atmosphäre auf eine Temperatur größer als 400°F (204,44°C), um eine im Wesentlichen chromfreie, Silizium enthaltende Schutzschicht (16) auf der Oberfläche (14) auszubilden, die Silizium aus der angetrockneten, Silizium enthaltenden Fluidkomposition und Metall aus der Metallkomponente (10) enthält.

2. Beschichtungsverfahren nach Anspruch 1, das des Weiteren umfasst Kombinieren der Siliziumwasserstoff-Flüssigkeit mit einer Dotiersubstanz, die aus der Gruppe bestehend aus Yttrium, Hafnium und Kombinationen davon ausgewählt ist.

3. Beschichtungsverfahren nach Anspruch 1 oder 2, wobei die im Wesentlichen chromfreie Metallkomponente (10) aus Eisen, Aluminium, Titan, Kupfer, Nickel oder einer Legierung dieser Stoffe besteht.

## Revendications

1. Procédé de revêtement destiné à protéger une surface (14) d'un composant métallique sensiblement exempt de chrome (10), comprenant l'application d'une couche (12) d'une composition de fluide au silicium sensiblement exempte de chrome comprenant un silane liquide sur au moins une partie de la surface (14), le durcissement de la composition de fluide au silicium sensiblement exempte de chrome après que la couche (12) est appliquée sur la surface (14), la mise en place de la composition de fluide au silicium dans une atmosphère non oxydante puis le chauffage de la composition de fluide au silicium sensiblement exempte de chrome durcie de la couche (12) dans l'atmosphère non oxydante à une température supérieure à 400 °F (204,44 °C) pour former un revêtement protecteur au silicium sensiblement exempt de chrome (16) sur la surface (14) qui inclut du silicium provenant de la composition de fluide au silicium durcie et un métal provenant du composant métallique (10).

2. Procédé de revêtement selon la revendication 1 comprenant en outre la combinaison du silane liquide avec un dopant choisi dans le groupe constitué de l'yttrium, de l'hafnium et de leurs combinaisons.

3. Procédé de revêtement selon la revendication 1 ou la revendication 2 dans lequel le composant métallique sensiblement exempt de chrome (10) est composé de fer, d'aluminium, de titane, de cuivre, de nickel, ou d'un alliage de ces matériaux.
